

1

2,793,113

## CREEP RESISTANT STEEL

John R. Rait and John O. Ward, Sheffield, England, assignors to Hadfields Limited, Sheffield, England

No Drawing. Application August 20, 1953,  
Serial No. 375,562

Claims priority, application Great Britain August 22, 1952

4 Claims. (Cl. 75—128)

This invention relates to ferritic alloy steels having improved resistance to scaling and creep deformation at high temperatures.

By a ferritic alloy we mean one which consists of an iron-rich matrix with excess carbide or other compounds as dispersed particles. Compounds, other than carbides, which may be present include nitrides, borides, and intermetallic compounds such, for example, as FeCr commonly referred to as "sigma phase" in ferrous alloys having high chromium contents. The matrix is usually in the body-centred cubic condition but may be more or less distorted by heat treatment; for example, after a very rapid cool, it may take the tetragonal form known as martensite. Such an alloy is magnetic at room temperature and will, on heating, transform into the non-magnetic face-centred cubic condition known as austenite and revert to the magnetic form on cooling. Some ferritic steels are hardenable by heat-treatment; others are not. When hardened, they may assume a variety of forms known as martensite, bainite, troostite, sorbite, pearlite, and so on. One ferritic alloy which has been proposed for service at high temperatures up to about 700° C. has a chromium content of 3% and consists principally of carbide formers and ferrite strengtheners, no attention being given to scale resistance. An example of it is shown at A in the following table:

5 When the chromium content of such alloys is increased to 12% we have found, and it is now commonly known, that the scaling resistance is greatly improved. The alloy then, however, has a very poor creep resistance as can be seen from example B in the table. We have found this to be due to the fact that, no matter how the alloy is heat treated, the presence of 12% chromium in the alloy prevents the formation of the face-centred cubic carbide, that is, vanadium carbide which is normally present when a smaller proportion of chromium is used and, in fact, leads to the formation of two chromium types of carbides, one having a trigonal structure and the other a complex cubic structure. The use of other elements forming face-centred cubic carbides has, therefore, been tried such, for example, as the 12% chromium alloy containing niobium shown at C in the table. A substantially increased creep resistance has thus been obtained but one which still gives scope for much improvement.

15 It is well known that the desirable treatment of such alloys consists of a high temperature solution treatment followed by a tempering or ageing treatment. For example, the solution treatment may be carried out above 1150° C. provided the temperature employed avoids overheating, burning, or excessive grain coarsening. It is also well known that the addition of 12% chromium to iron decreases the temperature and composition ranges at which austenite is stable. Since the creep resistance properties of these alloys depend on the different solubilities 20 of carbon in ferrite and austenite, an alloy which does not become wholly austenitic at the solution treatment temperature but develops a duplex ferritic-austenitic structure, cannot develop its optimum properties. The alloy shown at C in the table is prone to form this duplex structure on heating to the desired temperatures for carbide solution. The ferritic tendency may be avoided 25 by the addition of nitrogen or nickel or other austenitizing elements and a very substantial increase in creep resistance be thereby obtained as can be seen from the alloy shown at D in the table.

30 Whereas the cubic carbide has formerly been provided

Table

|          | Analysis |      |    |       |     |       |       |       | Total Creep Deformation, percent at times stated under a tensile stress of 8 tons/sq. in. at 600° C. |         | Comparative Creep Resistance based on 8 tons/sq. in. at 600° C. and 300 hrs. |     |
|----------|----------|------|----|-------|-----|-------|-------|-------|------------------------------------------------------------------------------------------------------|---------|------------------------------------------------------------------------------|-----|
|          | C        | Cr   | Mo | W     | V   | Nb    | Ti    | N     | B                                                                                                    | 300 hrs | 1000 hrs                                                                     |     |
| (A)----- | .2       | 3.0  | .5 | .5    | .8  | ----- | ----- | ----- | -----                                                                                                | .130    | .250                                                                         | 100 |
| (B)----- | .2       | 12.0 | .5 | .5    | .8  | ----- | ----- | ----- | -----                                                                                                | .500    | -----                                                                        | 28  |
| (C)----- | .16      | 12.0 | .5 | ----- | .6  | .15   | ----- | ----- | -----                                                                                                | .159    | .400                                                                         | 82  |
| (D)----- | .16      | 12.0 | .5 | ----- | .3  | .3    | ----- | .1    | .03                                                                                                  | .073    | .116                                                                         | 178 |
| (E)----- | .16      | 12.0 | .5 | ----- | .16 | .16   | .16   | .1    | .03                                                                                                  | .065    | .104                                                                         | 200 |
| (F)----- | .16      | 12.0 | .5 | ----- | .16 | .16   | .16   | .1    | .03                                                                                                  | .053    | .078                                                                         | 243 |

The alloy shown at A and, generally speaking, all similar ferritic alloys with good creep resistance have poor scaling resistance.

It has been clearly shown in published work that if such an alloy is to have a good creep resistance at high temperatures, its composition must be adjusted so that the optimum amount of carbide of a face-centred cubic structure is formed, i. e. so that the carbides present have a structure similar to that of sodium chloride. The creep resistance is dependent upon the combination of the constitution of the matrix, the crystal form, size distribution and composition of the carbides, these factors being dependent upon the manner in which the alloy is heat treated.

60 by two carbide formers, i. e. niobium and vanadium, we find that a mixture of three or more face-centred cubic carbides is preferable. The carbide formers can, for example, be titanium, vanadium, and niobium. The use of titanium enables a reduced amount of niobium and vanadium to be employed with a further substantial increase in creep resistance—see the alloy shown at E in the table. A still further increase in creep resistance is obtained by the addition of boron as shown at F in the table.

65 The use of titanium as a carbide former is of the greatest importance both technically and commercially. Technically, as can be seen from the table, it leads to a very substantial increase in creep resistance. Commercially,

its importance is that it is both cheap and abundant in comparison with niobium and tantalum and, as its use allows the amounts of the latter elements to be substantially reduced, it has a substantial bearing on the cost of production of the alloys.

The addition of the titanium is preferably made as titanium metal to the molten steel after deoxidation of the bath by means of calcium-silicon-zirconium or other suitable deoxidant. Ferro-titanium may be used but the titanium metal is preferred since ferro-titanium commonly contains impurities which may have a deleterious effect on the creep resistance.

The table given above gives in Examples E and F the analysis of particular alloys in accordance with the invention and is concerned only with essential elements. In general, the invention extends to ferritic steel alloys having high creep resistance and scaling resistance at temperatures up to about 700° C. and having as essential constituents:

|                                                                                                                              | Percent    | 20 |
|------------------------------------------------------------------------------------------------------------------------------|------------|----|
| Carbon                                                                                                                       | 0.05-0.50  |    |
| Chromium                                                                                                                     | 8.0-17.0   |    |
| Molybdenum                                                                                                                   | $\geq 4.0$ |    |
| or                                                                                                                           |            |    |
| Tungsten                                                                                                                     | $\geq 2.0$ |    |
| or                                                                                                                           |            |    |
| Molybdenum                                                                                                                   | $\geq 4.0$ |    |
| Tungsten                                                                                                                     | $\geq 4.0$ |    |
| Nitrogen                                                                                                                     | 0.01-0.25  | 30 |
| Silicon                                                                                                                      | 0.1-2.0    |    |
| Manganese                                                                                                                    | 0.1-4.0    |    |
| Three or more carbide formers including titanium and selected from vanadium, niobium, tantalum, titanium, hafnium, zirconium | 0.05-4.0   | 35 |

The alloys may also usefully contain:

|        | Percent     | 40 |
|--------|-------------|----|
| Nickel | $\geq 2.0$  |    |
| Boron  | $\geq 0.5$  |    |
| Cobalt | $\geq 10.0$ |    |
| Copper | $\geq 2.0$  |    |

A typical percentage composition would be:

|                             |       |
|-----------------------------|-------|
| Carbon                      | 0.15  |
| Silicon                     | 0.57  |
| Manganese                   | 0.85  |
| Chromium                    | 10.6  |
| Nickel                      | 0.09  |
| Molybdenum                  | 0.55  |
| Vanadium                    | 0.19  |
| Niobium and tantalum        | 0.19  |
| Titanium                    | 0.15  |
| Boron                       | 0.030 |
| Nitrogen                    | 0.094 |
| Copper                      | 0.13  |
| And unavoidable impurities. |       |

The heat treatment of such an alloy should comprise a high temperature treatment followed by a tempering or ageing treatment.

The alloys in accordance with the invention can be used under high stress and high temperature conditions such as occur in gas turbines and other applications.

The following is a typical example of results obtained from the invention:

A disc approximately 24 inches in diameter and 2 inches thick with an integral boss 8 inches in diameter and  $4\frac{1}{2}$  inches thick was forged from an ingot 15 inches square of a steel manufactured by the basic electric arc process having the following percentage composition:

|      |       |
|------|-------|
| C    | 0.16  |
| Si   | 0.42  |
| Mn   | 1.17  |
| Cr   | 10.4  |
| 5 Ni | 0.20  |
| Mo   | 0.52  |
| V    | 0.25  |
| Ti   | 0.11  |
| B    | 0.015 |
| 10 N | 0.054 |
| Cu   | 0.16  |
| W    | <0.01 |
| Co   | <0.03 |
| Nb   | 0.20  |

15 The disc was quenched from 1250° C. and tempered for 48 hours at 650° C. It was then found to have the following properties:

|                                                                                           | Tangential | Radial | Transverse at centre |
|-------------------------------------------------------------------------------------------|------------|--------|----------------------|
| Creep Deformation (percent) under a tensile stress 8 tons/sq. in. at 300 hours at 600° C. | 0.073      | 0.078  | 0.081                |
| 25 Tensile Strength at room temperature (tons/sq. in.):                                   |            |        |                      |
| 0.1% proof stress                                                                         | 52.4       | 51.6   | 49.9                 |
| max. stress                                                                               | 62.9       | 62.2   | 60.0                 |
| Elongation (percent) ( $L=4\sqrt{A}$ )                                                    | 15.5       | 15.0   | 15.0                 |
| Reduction of Area (percent)                                                               | 42.9       | 37.9   | 41.3                 |

We claim:

1. A ferritic alloy steel having high scale resistance and creep resistance up to about 700° C. and having as essential constituents:

|           | Percent   |
|-----------|-----------|
| Carbon    | 0.05-0.50 |
| Chromium  | 8.0-17.0  |
| Nitrogen  | 0.01-0.25 |
| Silicon   | 0.1-2.0   |
| Manganese | 0.1-4.0   |

a substance selected from the group consisting of molybdenum (not greater than 4%), tungsten (not greater than 2%) and molybdenum tungsten (not greater than 4%), from 0.05 to 4% of at least three face centered cubic carbide formers including titanium and selected from the group consisting of titanium, vanadium, niobium, tantalum, hafnium, and zirconium, and the remainder being essentially iron.

2. A ferritic alloy steel according to claim 1 containing also any one or more of the following:

|        | Percent     |
|--------|-------------|
| Nickel | $\geq 2.0$  |
| Boron  | $\geq 0.5$  |
| Cobalt | $\geq 10.0$ |
| Copper | $\geq 2.0$  |

3. A ferritic steel alloy having the percentage composition:

|           |      |
|-----------|------|
| Carbon    | 0.15 |
| Silicon   | 0.57 |
| Manganese | 0.85 |
| Chromium  | 10.6 |
| Nickel    | 0.09 |

|                      |       |
|----------------------|-------|
| Molybdenum           | 0.55  |
| Vanadium             | 0.19  |
| Niobium and tantalum | 0.19  |
| Titanium             | 0.15  |
| Boron                | 0.030 |

|                             |       |
|-----------------------------|-------|
| Nitrogen                    | 0.094 |
| Copper                      | 0.13  |
| And unavoidable impurities. |       |

4. A ferritic alloy steel containing 0.05-0.50% carbon, 8.0-17.0% chromium, a substance selected from the group consisting of molybdenum (not greater than 4%),

tungsten (not greater than 2%) and molybdenum tungsten (not greater than 4%), from 0.05 to 4% of at least three face centered cubic carbide formers including titanium and selected from the group consisting of titanium, vanadium, niobium, tantalum, hafnium, and zirconium, the balance substantially iron.

## References Cited in the file of this patent

## UNITED STATES PATENTS

- |           |               |       |               |
|-----------|---------------|-------|---------------|
| 2,542,220 | Urban         | ----- | Feb. 20, 1951 |
| 2,576,229 | Krainer       | ----- | Nov. 27, 1951 |
| 2,590,835 | Kirkby et al. | ----- | Apr. 1, 1952  |